

## UNITED STATES PATENT OFFICE.

FRANK S. LOW, OF NIAGARA FALLS, NEW YORK.

## TANNING.

No Drawing.

Application filed August 13, 1925. Serial No. 50,137.

This invention relates to tanning; and it comprises a method of converting hide into leather wherein a tanning bath is produced by the solution of an anhydrous chromium chlorid in water, this chlorid being sometimes chromous chlorid but more frequently chromic chlorid in the presence of some chromous chlorid or of a reducing body adapted to form chromous chlorid, such as 5 ferrochrome, untanned hides being treated by such a bath; all as more fully hereinafter set forth and as claimed.

Chromium has three states of oxidation, chromium trioxid,  $\text{CrO}_3$  (chromic acid); 15 chromic oxid (sesquioxid)  $\text{Cr}_2\text{O}_3$ , and chromous oxid,  $\text{CrO}$ . As will be noted, the ratio of oxygen to chromium in the trioxid is twice as great as in chromic oxid; and that in chromous oxid is two-thirds that in 20 chromic oxid. In recovering chromium from its ore, chrome iron stone, it is usual to roast the ore in the presence of air and alkali, thereby oxidizing the contained  $\text{Cr}_2\text{O}_3$  to form a chromate with the alkali 25 present, this chromate being afterwards leached out. From the chromate other chromium compounds are prepared, if wanted. In chrome tanning, the active agent is  $\text{Cr}_2\text{O}_3$  which is taken up from slightly basic 30 solutions by hide with the production of leather; the expression " $\text{Cr}_2\text{O}_3$ " being used for convenience and without theory as to whether it is actually " $\text{Cr}_2\text{O}_3$ " or some hydrated form of the oxid in solution or col- 35 loidal suspension or forms a component of a basic salt. Not much is actually known as to this. Chrome tanning can be effected by the use of a bichromate, usually sodium bichromate. The  $\text{CrO}_3$  of the chromate is 40 converted into  $\text{Cr}_2\text{O}_3$  by reduction. As a reducing agent, glucose is sometimes added, together with sulfuric acid to combine with the base of the chromate. In making chrome tanning baths, sodium bichromate 45 has the advantage of being a primary commercial material, other chromium compounds being usually made from it, and the further advantage that it is a definite salt, not of a hygroscopic nature and is easily 50 packaged, shipped and handled. But in the tan bath, it must undergo complex changes and the bath becomes loaded with inert products of reaction.

In tanning, whatever the theory of the 55 action that occurs, a bath which will tan

invariably contains a salt of chromium in the state of oxidation corresponding to chromic oxid; this salt containing less of the negative radicle ( $\text{Cl}$ ,  $\text{SO}_4$ , etc.) than corresponds to the normal salts,  $\text{CrX}_3$ . In 60 other words, a basic salt is present; this salt being usually considered  $\text{CrX}_2\text{OH}$  in which  $\text{X}$  denotes a negative radicle.

For the present purposes, dissolved chromic salts, such as the sulfate and chlorid, 65 may be considered as  $\text{Cr}_2\text{O}_3$  held in solution by the corresponding acid. From a salt containing the full theoretical amount of acid, namely  $6\text{HCl}$  or  $3\text{H}_2\text{SO}_4$  for each  $\text{Cr}_2\text{O}_3$ , hide takes up but little  $\text{Cr}_2\text{O}_3$ . In 70 a way, tanning may be considered as a sort of competition between hide substance and acid for  $\text{Cr}_2\text{O}_3$  and the best tanning results are obtained from solutions in which the amount of acid is about two-thirds that 75 theoretically required by the  $\text{Cr}_2\text{O}_3$ ; that is, from a basic salt which may be regarded at pleasure as  $\text{Cr}_2\text{O}_3\cdot 4\text{HCl}$  or  $\text{Cr}_2\text{Cl}_4(\text{OH})_2$  or  $\text{CrCl}_2\cdot \text{OH}$ . The three formulas all mean the same thing—a basic chromic salt. Such 80 a salt is produced in the course of all tanning processes and as its basicity lessens with fixing of  $\text{Cr}_2\text{O}_3$  by the hide, small amounts of soda ash are added to restore the basic condition.

It is one of the objects of the present invention to enable the tanner to produce directly such a bath containing a basic chromium salt and capable of tanning from the start without the necessity of initially adding bases, acids, glucose, etc.

While the chromates have the advantage that they are relatively cheap, pure and easily obtainable, they present certain disadvantages in this relation. In use, there is 95 a necessary reduction of chromium trioxid to sesquioxid before tanning can be done; and an adjustment of base-and-acid relations. For various reasons, chromium chlorid is a more desirable body for making 100 the tanning baths, but unfortunately it has not been possible to obtain it readily in a pure state. Its manufacture from bichromate is an unnecessary complication and, moreover, it is not readily obtained pure and 105 dry. The commercial hydrated chlorid,  $\text{CrCl}_3\cdot 6\text{H}_2\text{O}$ , is an extremely hygroscopic material; difficult to make, ship and handle; or to prepare of any definite chromium content; and before it can be used its solutions 110

must be treated with alkali to obtain a basicchlorid. On treating this mixture with hot salt.

I have found that excellent results can be obtained in using as a material for tanning baths an anhydrous chromium chlorid prepared in the dry way; this chromium chlorid being either  $\text{CrCl}_3$  or  $\text{CrCl}_2$  or a mixture of the two. Upon exposure to chlorin at a proper temperature, ferro-chrome is converted into solid chromium chlorid and ferric chlorid, the latter vaporizing. By this method, it is easy to prepare either chromous or chromic chlorid in a state of purity. Anhydrous chromic chlorid, free from chromous chlorid, is a purple or violet crystalline mass which is insoluble in water and is readily stored, shipped and handled. It is not in any way corrosive to metals and there is no difficulty in packaging it. In these respects it has the advantage over any commercial hydrated form of chlorid. In the presence of a little chromous chlorid, anhydrous chromic chlorid becomes soluble in water; the proportion of chromous chlorid necessary to effect this being extraordinarily little. In making chromic chlorid, it is practicable to turn out a product containing this small amount. Such a product while having all the other properties and advantages of the anhydrous purple chlorid just described, can be readily dissolved in water. With chromic chlorid the tanner can readily make pure baths of definite composition which however require addition of a little alkali to produce a basic salt.

Chromous chlorid is a yellow micaceous material soluble in water. Its solutions in water readily oxidize to the chromic form and give a basic chromic chlorid containing two-thirds the chlorin necessary for normal chromic chlorid; in other words, giving solutions at once adapted for tanning.

In the present invention, these anhydrous chromium chlorids may be utilized in various ways in making standardized definite tanning baths without the necessity and nuisance of the use of glucose and sulfuric acid. The anhydrous purple chromic chlorid in its insoluble form can be shipped and stored, as stated, without trouble and can be readily brought into solution by the tanner by the use of a little reducing agent of any kind; something which will form chromous chlorid. Zinc may be used. Incidentally, zinc as a reducing agent disposes of part of the chlorin and the solution formed is to that extent equivalent to an oxychlorid. The soluble form has practically the same advantages but requires no addition of reducing agent since it already contains some (chromous chlorid).

A very simple and efficient way of making a tanning bath is to use a mixture of fine ground ferrochrome and anhydrous chromic

water, the chromium of both bodies goes into solution readily with production of chromous chlorid; this chromous chlorid oxidizing swiftly to chromic chlorid. Since however the ratio of chlorin to chromium in chromous chlorid,  $\text{CrCl}_2$ , is only two-thirds that obtaining in chromic chlorid,  $\text{CrCl}_3$ , in oxidizing a basic chlorid or oxychlorid is formed. The bath formed from a mixture of ferrochrome and chromic chlorid is a tanning bath which tans without necessity for a preliminary introduction of alkali. It is only necessary to add alkali as exhaustion of the bath progresses. Exactly the same considerations apply when chromous chlorid itself is employed as a tanning bath. The  $\text{CrCl}_2$  quickly takes up oxygen and is converted into the equivalent of  $\text{Cr}_2\text{Cl}_4\text{O}$ , or a soluble basic chlorid.

Aside from their convenient physical nature, the preparations in question have the advantage of offering the tanner something which can be made of definite composition as regards chromium content and which is very rich in chromium. The  $\text{Cr}_2\text{O}_3$  equivalent of chromic chlorid is about the same as that of sodium bichromate, while that of chromous chlorid or of a mixture of chromic chlorid and ferrochrome is considerably higher.

In operating under the present invention, the preparation of tanning baths is exceedingly simple. Anhydrous chromous chlorid in the desired amount may be dissolved in hot water and the bath directly used. Basic chromic chlorid is formed as rapidly as hide will take up  $\text{Cr}_2\text{O}_3$ . Additions of soda are made from time to time after the first tanning action is complete. Or, in lieu of using chromous chlorid directly, the anhydrous chromic chlorid may be placed in hot water with a little zinc or a little finely ground ferrochrome and the solution directly used as a tanning bath. For the convenience of the tanner, it is possible to furnish a fine ground preparation of anhydrous insoluble chromic chlorid and fine ground ferrochrome. To obtain the maximum amount of chromous chlorid, using commercial ferrochrome, a ratio of 6 parts anhydrous chromic chlorid to 1 part of ferrochrome is advisable. However, considerably smaller amounts of metallic ferrochrome will suffice to render chromic chlorid soluble. The mixture on treatment with hot water goes into solution, giving a tanning bath. In this bath, using the full amount of ferrochrome, the chromium is mainly contained as chromous chlorid, which, however, quickly changes to the chromic form by oxidation, giving a solution of chromic oxychlorid. Oxidation may be hastened and facilitated by aerating the bath. In lieu of using ferrochrome, powdered zinc may be used, but there is no ad-

vantage in this substitution. The preparations mentioned may be made, shipped and stored commercially and directly used by the tanner. On the addition of water, the 5 described action takes place.

Tanning may be done in the usual ways, by drumming, etc. In drumming the agitation of the bath provides aeration.

What I claim is:-

- 10 1. In tanning hides and skin, the process which comprises exposing untanned hide to the action of a solution containing chromic and chromous chlorids.
- 15 2. In tanning hides and skins, the process which comprises exposing untanned hide to the action of a solution containing chromous chlorid.
- 20 3. In tanning hides and skins, the process which comprises forming a solution containing chromous chlorid and exposing untanned hide to the action of the resultant bath under conditions permitting oxidation of the chromous chlorid to basic chromic chlorid.
- 25 4. In tanning hides and skins, the process which comprises bringing anhydrous chromic chlorid into solution with the aid of a reducing agent and tanning untanned hide with the resultant bath under conditions

permitting oxidation of the chromous chlorid formed in the bath. 30

5. In tanning hides and skins, the process which comprises bringing anhydrous chromic chlorid into solution with the aid of ferrochrome and tanning untanned hide with the 35 resultant bath under conditions permitting oxidation of the chromous chlorid formed in the bath.

6. In tanning hides and skins, the process which comprises exposing untanned hide 40 to an aerated bath containing chromous chlorid.

7. In tanning hides to make leather the process which comprises submitting untanned hides to the action of a chromium 45 chlorid solution containing chromium in the chromous form.

8. As a new composition of matter for tanning purposes, a mixture of ferrochrome and anhydrous chromic chlorid. 50

9. A new composition of matter for tanning purposes, a mixture of anhydrous chromic chlorid and a metal capable of reducing it.

In testimony whereof, I have hereunto 55 affixed my signature.

FRANK S. LOW.